

3,206,362

## SETTING LOTION FOR HAIR

Jean Hollub, Geneva, Burkhardt Lange, Basel, and Arthur Maeder, Therwil, Switzerland, assignors to Ciba Limited, Basel, Switzerland, a company of Switzerland  
No Drawing. Filed July 3, 1963, Ser. No. 292,756  
Claims priority, application Switzerland, July 4, 1962,  
8,028/62

12 Claims. (Cl. 167—87.1)

It is known to use hairdressing preparations in order to maintain the hair in a desired shape. For this purpose there may be applied to the dry, combed hair a film-forming substance which has a setting effect on the hair. These preparations, also called hair lacquers, are primarily applied to the hair in the form of aerosol sprays. In this manner, depending on the amount of spray used, there is produced, especially on the outside, a coating of lacquer of varying thickness which by virtue of its inner strength has a setting and stiffening effect on the individual hairs. There are also known preparations which are applied to the damp hair in aqueous form. In this case the hair is advantageously rolled into the desired shape and then dried. In this method the damp hair is impregnated with the setting lotion and after drying all hairs are completely covered with a very thin film; the hair treated in this manner does not feel stiff as it usually does when sprays are applied to it, it has a soft feel and has been set in the desired style.

From German Auslegeschrift 1,084,440 it is known to use hairdressing preparations containing a basic polymer capable of forming salts, for example the chloride of the homopolymer of 2-vinyl-5-methylpyridine and of the acrylic acid diethylaminoethyl ester. However, after drying these salts form film that are soluble in water at room temperature. While their use in setting lotions does produce a setting coating on the hair, this coating is, because of its solubility in water, not resistant to moisture so that when the hair so treated is once more curled it can no longer be set in the original style. In a moist atmosphere any hair dressing preparation producing a non-moisture resistant film will migrate along the hairs and collect at the tips.

It has now been found that certain water-soluble salts of basic copolymers obtained by linear addition are rendered, by simple drying at temperatures ranging from 18 to 60° C. resistant to or soluble in water. Hair treated with such salts has the advantage that neither rain nor damp air will dissolve the coating. When hair treated with the setting lotion of the invention is exposed to moisture, then again laid in the desired style and dried, the resulting hairstyle is again stable as to shape. With known setting lotions based on dextrins, tragacanth, acrylic acid polymers, polyvinylpyrrolidone or the like do not produce this effect since the action of water or damp air on them washes them off. Although the setting lotions of the invention are resistant to moisture, it is easy to wash them out of the hair with a shampoo.

The basic copolymer to be used according to the invention must be composed so that it satisfies two essential requirements, namely it must be capable of forming salts that are soluble in water, and it must form a water-insoluble film when its aqueous solution is dried at 18 to 60° C.

The present invention provides a moisture-resistant setting lotion in the form of an aqueous or aqueous-alcoholic solution for setting hair that has been laid in the damp state, the said solution containing an amount of 0.5 to 5% of a salt, which is at least soluble in an aqueous-alcoholic solution, of a weak inorganic or organic acid and a basic copolymer capable of forming films; the copolymer contains at least an amount of a basic mono-

meric compound containing a tertiary nitrogen atom sufficient to ensure that after the hair has been dried at a temperature ranging from 18 to 60° C. a water-insoluble film is left on it. Furthermore, the present invention provides a method of making water waves of enhanced durability, more specially in a damp atmosphere, wherein damp hair is impregnated with an aqueous or aqueous-alcoholic solution containing 0.5 to 5% of a salt, which is at least soluble in an aqueous-alcoholic solution, of a weak inorganic or organic acid and a basic copolymer capable of forming films, the said copolymer containing a basic monomer with a tertiary nitrogen atom in an amount sufficient to ensure that after having been dried the hair is covered with a water-insoluble film, whereupon the impregnated hair is laid in the desired shape and dried at a temperature ranging from 20 to 60° C., preferably from 30 to 50° C.

The solubility of the salts in water must be such that they are soluble at 15 to 25° C. and at a concentration of 20 up to 20% by weight in water or in an aqueous-alcoholic mixture of 2 parts by weight of ethanol and at least 8 parts of water. If the share of the salt-forming, basic component is too large, drying does not convert the films into the water-insoluble state; if it is too small, no water-soluble salts are formed. The expert will be able to ascertain by simple tests the maximum and minimum amounts of basic component required to ensure the desired solubility of the salts in water and their capability of forming a water-insoluble film.

The solubility of the salts in water and their capability of forming water-insoluble films depend also on the kind and amount of the non-basic comonomers. When, for example, acrylamide or its N-substituted alkylacrylamides are used the share of the basic component may be smaller than when esters of acrylic or methacrylic acid are used. Since the manufacture of copolymers having the desired properties depends on a number of factors that affect one another, it is not possible to lay down a rule applicable to all cases. If the basic component used is an N:N-dialkylaminoalkyl acrylamide, it should as a rule be used in an amount not exceeding 30% by weight and not less than 5%. When an N:N-dialkylaminoalkyl methacrylic acid ester is used, the less pronounced solubilizing properties require 50% by weight or even more to be used.

As acids capable of forming salts there come into consideration weak inorganic or organic acids, that is to say acids whose dissociation constant is below  $10^{-3}$ . There may be mentioned: Boric, carbonic, formic, acetic, propionic and lactic acid. It is of special advantage to use a readily volatile acid, such as carbonic, formic or acetic acid.

To test the salts for their capability of forming water-insoluble films an aqueous solution of the salts is poured over a plate of glass and allowed to evaporate at 18 to 25° C. The film (film thickness about  $20\mu$ ) is then dried for 1 hour at 45° C. The film is then kept covered with water for 1 hour at 18 to 25° C., and its dissolution or stability respectively is ascertained.

As a rule, the setting lotions contain the salts described above in a concentration of 0.5 to 5%, preferably 0.75 to 2% by weight. The solvent used may be water or, more advantageously, it is a mixture of alcohol and water because the alcohol promotes the evaporation and drying. The aqueous preparation used as setting lotion may contain, apart from the solvent or solvents and the salt of the basic copolymer, the conventional additives such as perfume, softening agents, evaporation accelerators and the like. As relevant examples there may be mentioned higher monohydric alcohols with 6 to 18 carbon atoms, polyhydric alcohols such as ethyleneglycol and polyethyleneglycols, condensation products of ethyl-

ene oxide with compounds having an active hydrogen atom, and carbamides such as urea, ethylene urea and biuret. The setting lotions consist preferably of 0.75 to 2% of the salt of the basic copolymer, 0.5 to 3% of additives, 5 to 20% of ethanol and 95 to 75% of water. The manufacture of the salts and of the basic copolymers is known. The salts can be prepared from the free bases by adding a calculated amount of acid.

As basic polymerizable compounds, whose molecule contains at least one tertiary nitrogen atom, there are particularly suitable the compounds of the following types:

- (a) Basic amides or esters of aliphatic  $\alpha$ : $\beta$ -ethylenically unsaturated monocarboxylic or dicarboxylic acids with 3 to 5 carbon atoms;
- (b) Basic vinyl ethers.

The copolymers are particularly advantageous to manufacture from the compounds of type (a), especially from the basic acids of polymerizable aliphatic  $\alpha$ : $\beta$ -unsaturated monocarboxylic acids whose molecule contains a tertiary nitrogen atom in the amide constituent. The basic amides and esters are derived from an  $\alpha$ : $\beta$ -unsaturated acid of the acrylic acid series, that is to say from homologues of acrylic acid, such as methacrylic or crotonic acid, or from the corresponding dicarboxylic acids, such as fumaric, itaconic or citraconic acid.

The basic amides and esters of monocarboxylic acids correspond preferably to the general formula



where X represents a hydrogen atom or the methyl group, n and s each is 1 or 2, and R<sub>1</sub> and R<sub>2</sub> each stands for an alkyl radical with 1 to 4 carbon atoms. R<sub>1</sub> and R<sub>2</sub> may also be linked together to form a heterocycle. When n=1, the formula represents an amide of a copolymerizable acid; when n=2 it stands for a corresponding ester. As examples of basic amides of the Formula 1 there may be mentioned:

Acrylic acid- $\gamma$ -diethylaminopropylamide,  
Methacrylic acid- $\gamma$ -dimethylaminopropylamide,  
Methacrylic acid- $\beta$ -diethylaminoethylamide,  
Acrylic acid- $\beta$ -dimethylaminoethylamide,  
Acrylic acid- $\beta$ -N-morpholinoethylamide, and  
Acrylic acid- $\beta$ -pyrrolidinoethylamide.

As examples of basic esters of the Formula 1 there may be mentioned:

Acrylic acid- $\beta$ -diethylaminoethyl ester,  
Acrylic acid- $\beta$ -dimethylaminoethyl ester,  
Methacrylic acid- $\gamma$ -diethylaminopropyl ester, and  
Acrylic acid- $\gamma$ -di-n-butylaminopropyl ester.

Compounds of the type (a) may also be basic amides or esters of aliphatic  $\alpha$ : $\beta$ -unsaturated dicarboxylic acids, such as maleic acid- $\gamma$ -dimethylaminopropylamide, fumaric acid-di-[ $\gamma$ -dimethylaminopropyl]-amide and fumaric acid-di-[ $\beta$ -diethylaminoethyl]-ester.

As examples of the basic vinyl ethers mentioned under (b) there may be used vinyl ethers containing a tertiary nitrogen atom and up to 12 carbon atoms, specifically the following:  $\beta$ -diethylaminoethyl vinyl ether,  $\beta$ -di-n-butylaminoethyl vinyl ether,  $\beta$ -morpholinoethyl vinyl ether and 4-dimethylaminophenyl-(1)-methylvinyl ether.

The manufacture of the basic monomers to be used according to this invention is known and does not form an object of the invention.

The polymerization may be conducted in solution or in emulsion, using the measure conventionally employed in the polymerization technique. Preferably, the polymerization is performed in solution. The basic copolymers may be manufactured by the processes described in the British patent application No. 871,295, granted October 18, 1961, by A. Maeder, and British patent application No. 75

876,674, granted December 27, 1961, by A. Maeder. To convert the basic polymer into the salt, the polymer solution is concentrated by evaporating the solvent, whereupon advantageously the calculated amount of acid is added and the whole is diluted with water. When the salt to be manufactured is the carbonate, the solution is freed from the solvent and diluted with water and carbon dioxide is injected into it while cooling with ice.

As monomers with which the basic monomers are to be copolymerized there are suitable non-basic compounds which likewise contain a carbon-to-carbon double bond, more especially an  $\text{H}_2\text{C}=\text{C}$  group, in particular vinyl esters of organic acids, for example vinyl acetate, formate, butyrate or benzoate, or vinylaryl compounds such as styrene or substituted styrenes, compounds of the acrylic acid series such as esters of acrylic acid and alcohols or phenols that contain 1 to 12 carbon atoms and no tertiary amino group, for example ethyl acrylate, butyl acrylate and dodecyl acrylate, acrylonitrile or acrylamide and its derivatives substituted on the amide nitrogen, such as N:N-diethyl acrylamide, N:N-dihydroxyethyl acrylamide, N-n-propyl acrylamide, N-tertiary butyl acrylamide, N:N-di-n-butyl-acrylamide and hexamethyolmelamine triacrylamide; furthermore, analogous derivatives of methacrylic,  $\alpha$ -chloracrylic, crotonic, maleic or fumaric acid. There may also be used polymerizable vinyl ethers such as vinylethyl ether. Preferred use is made of derivatives of acrylic and methacrylic acid (said derivatives being free from basic nitrogen atoms) and among them above all the esters with aliphatic alcohols, or the N-monosubstituted amides in which an aliphatic substituent is linked to the amide nitrogen atom through a secondary or tertiary carbon atom. Particularly suitable are ternary copolymers that contain as the film-forming component 30 to 50% of an ester of acrylic or methacrylic acid and an alkanol with 1 to 4 carbon atoms; as setting and sheen-forming component 30 to 50% of an N-monoalkyl-substituted or N:N-dialkyl-substituted acrylamide whose substituents contain 2 to 4 carbon atoms each, and as salt-forming component 5 to 20% of an N:N-di-(C<sub>2</sub>-C<sub>3</sub>) alkylamino-(C<sub>2</sub>-C<sub>3</sub>) alkylacrylamide.

Percentages in the following examples are by weight.

#### Example 1

45 160 parts of ethyl acrylate, 200 parts of N-tertiary butyl acrylamide and 40 parts of N:N-diethylaminopropyl acrylamide are dissolved at room temperature in 320 parts of absolute ethanol in a 2-filter flask equipped with stirrer, reflux condenser and thermometer. The flask is then scavenged with nitrogen and the batch is heated to the boiling point of ethanol. 0.4 part of azo diisobutyronitrile is then added, and this addition is repeated four times at intervals of 1 hour each. The polymerization is slightly exothermic. 1 hour after the last addition of catalyst the mixture is cooled to room temperature.

50 Yield: 710 parts of a low viscous, colorless and clear resin solution having a solids content of 56%, which corresponds to a polymer yield of almost 100%.

55 The resin solution is mixed with 14.5 parts of acetic acid (100%), and 1265 parts of deionized water are slowly run in. The resulting thinly viscous, opalescent solution is filtered through a clarifying filter.

60 Yield: about 2000 parts, solids content 20.5%, pH=5.5.

When the solution is poured over a glass plate and allowed to dry in air, it forms a transparent, colorless film which, after having been stored for 72 hours at 18° C., still remains completely insoluble on immersion for 60 minutes in water at 18° C.

#### Example 2

70 Setting lotions are prepared with the use of the undermentioned salts, having the following composition:

1.25% of a salt of a copolymer Nos. 1 to 14,  
0.4% of hexanol,  
0.1% of urea,

0.6% of a condensation product from 1 mol of stearyl alcohol and 25 mols of ethylene oxide,  
10% of alcohol,  
made up to 100% with water.

The salts concerned are the following products:

- (1) Formate salt of the copolymer from 40% of ethyl acrylate, 55% of N-tertiary butyl acrylamide and 5% of N:N-diethylaminomethacrylate.
- (2) Acetate salt of the copolymer from 90% of ethyl acrylate and 10% of N:N-diethylaminopropyl acrylamide.
- (3) Acetate salt of the copolymer from 50% of ethyl acrylate, 40% of N-tertiary butyl acrylamide and 10% of N:N-diethylaminopropyl acrylamide.
- (4) Acetate salt of the copolymer from 80% of ethyl acrylate, 10% of N-tertiary butyl acrylamide and 10% of N:N-diethylaminopropyl acrylamide.
- (5) Propionate salt of the copolymer from 80% of ethyl acrylate and 20% of N:N-diethylaminopropyl acrylamide.
- (6) Acetate salt of the copolymer from 40% of ethyl acrylate, 50% of N:N-di-n-butyl acrylamide and 10% of N:N-diethylaminopropyl acrylamide.
- (7) Carbonate salt of the copolymer from 85% of n-butyl acrylate and 15% of N:N-dimethylaminoethyl acrylamide.
- (8) Borate salt of the copolymer from 70% of methyl acrylate and 30% of N:N-diethylaminopropyl acrylamide.
- (9) Lactate salt of the copolymer from 30% of ethyl acrylate, 10% of lauryl acrylate, 40% of N:N-diethyl acrylamide and 20% of N:N-diethylaminoethyl acrylamide.
- (10) Acetate salt of the copolymer from 40% of methyl methacrylate, 40% of n-butyl acrylate and 20% of N:N-diethylaminopropyl methacrylamide.
- (11) Propionate salt of the copolymer from 50% of methyl acrylate, 15% of vinyl acetate and 35% of diethylaminopropyl vinyl ether.
- (12) Acetate salt of the copolymer from 40% of ethyl acrylate, 30% of N-tertiary butyl acrylamide and 30% of N:N-diethylaminoethyl vinyl ether.
- (13) Formate salt of the copolymer from 30% of ethyl acrylate, 20% of N-tertiary butyl acrylamide and 50% of N:N-diethylaminoethyl methacrylate.
- (14) Acetate salt of the copolymer from 75% of ethyl acrylate and 25% of di-(N:N-dimethylaminopropyl)-fumaric acid amide.

The hair is thoroughly washed and then dried with a towel only so much as to leave it damp. 10 to 30 ml. of setting lotion are then applied so as to leave the hair thoroughly damp. The hair is then given the desired style (preferably by curling) and dried in air heated up to 40° C. In all 14 cases there are obtained water waves which display a coating that is resistant to moist air. The hair can be styled again in the damp state and without additional treatment, and the resulting hairstyle is permanent.

What is claimed is:

1. A composition for setting hair that has been shaped in the damp state, comprising a solvent selected from the class consisting of water and a mixture of water and alcohol, and, in an amount of 0.5 to 5 percent, calculated on the total of the solution, a salt which is soluble in said solvent, of a weak acid selected from the group consisting of boric acid, carbonic acid, formic acid, acetic acid, propionic acid and lactic acid and a basic, film-forming copolymer, said copolymer consisting of (1) 30 to 50 percent by weight of units of an alkyl ester of an acid selected from the group consisting of acrylic and methacrylic acid, wherein the alkyl has 1 to 4 carbon atoms, (2) 30 to 50 percent by weight of units of a substituted acrylamide selected from the group consisting of N-mono-alkyl-substituted and N:N-dialkyl-substituted

acrylamide, the substituents containing 2 to 4 carbon atoms each, and (3) 5 to 20 percent by weight of units of an N:N-dialkyl-amino-alkylacrylamide, wherein the alkyl radicals contain at least 2 and at most 3 carbon atoms.

5 2. A composition for setting hair that has been shaped in the damp state, comprising a solvent selected from the class consisting of water and a mixture of water and alcohol, and, in an amount of 0.5 to 5 percent, calculated on the total of the solution, a salt which is soluble in said solvent, of acetic acid and a basic, film-forming copolymer, said copolymer consisting of 30 to 50 percent by weight of units of ethyl-acrylate, 30 to 50 percent by weight of units of N-tertiary butyl-acrylamide, and 5 to 20 percent by weight of units of N:N-diethylamino-propyl-acrylamide.

10 3. A composition for setting hair that has been shaped in the damp state, comprising a solvent selected from the class consisting of water and a mixture of water and alcohol, and, in an amount of 0.5 to 5 percent, calculated on the total of the solution, a salt which is soluble in said solvent, of acetic acid and a basic, film-forming copolymer, said copolymer consisting of 40% of ethyl acrylate, 30% of N-tertiary butyl acrylamide and 30% of N:N-diethylaminoethyl vinyl ether.

15 4. A composition for setting hair that has been shaped in the damp state, comprising a solvent selected from the class consisting of water and a mixture of water and alcohol, and, in an amount of 0.5 to 5 percent, calculated on the total of the solution, a salt which is soluble in said solvent, of acetic acid and a basic, film-forming copolymer, said copolymer consisting of 30% of ethyl acrylate, 20% of N-tertiary butyl acrylamide and 50% of N:N-diethylaminoethyl methacrylate.

20 5. A composition for setting hair that has been shaped in the damp state, comprising a solvent selected from the class consisting of water and a mixture of water and alcohol, and, in an amount of 0.5 to 5 percent, calculated on the total of the solution, a salt which is soluble in said solvent, of acetic acid and a basic, film-forming copolymer, said copolymer consisting of 75% of ethyl acrylate and 25% of di-(N:N-dimethylaminopropyl)-fumaric acid amide.

25 6. A method for making water waves of enhanced durability in a damp atmosphere, wherein the damp hair is impregnated with a composition as claimed in claim 1, the impregnated hair is laid in the desired shape and dried at a temperature ranging from 20 to 60° C.

30 7. A method for making water waves of enhanced durability in a damp atmosphere, wherein the damp hair is impregnated with a composition as claimed in claim 2, the impregnated hair is laid in the desired shape and dried at a temperature ranging from 20 to 60° C.

35 8. A method for making water waves of enhanced durability in a damp atmosphere, wherein the damp hair is impregnated with a composition as claimed in claim 3, the impregnated hair is laid in the desired shape and dried at a temperature ranging from 20 to 60° C.

40 9. A method for making water waves of enhanced durability in a damp atmosphere, wherein the damp hair is impregnated with a composition as claimed in claim 4, the impregnated hair is laid in the desired shape and dried at a temperature ranging from 20 to 60° C.

45 10. A method for making water waves of enhanced durability in a damp atmosphere, wherein the damp hair is impregnated with a composition as claimed in claim 5, the impregnated hair is laid in the desired shape and dried at a temperature ranging from 20 to 60° C.

50 11. A composition for setting hair that has been shaped in the damp state, comprising a solvent selected from the class consisting of water and a mixture of water and alcohol and, in an amount of 0.5 to 5 percent, calculated on the total of the solution, a salt which is soluble in said solvent, of lactic acid and a basic, film-forming copolymer, said copolymer consisting of 30 to 50 percent

by weight of units of ethyl-acrylate, 30 to 50 percent by weight of units of N-tertiary butyl-acrylamide, and 5 to 20 percent by weight of units of N:N-diethylamino-propyl-acrylamide.

12. A composition for setting hair that has been shaped in the damp state, comprising a solvent selected from the class consisting of water and a mixture of water and alcohol and, in an amount of 0.5 to 5 percent, calculated on the total of the solution, a salt which is soluble in said solvent, of formic acid and a basic, film-forming copolymer, said copolymer consisting of 30 to 50 percent by weight of units of ethyl-acrylate, 30 to 50 percent by

5

10

weight of units of N-tertiary butyl-acrylamide, and 5 to 20 percent by weight of units of N:N-diethylamino-propyl-acrylamide.

#### References Cited by the Examiner

##### UNITED STATES PATENTS

|           |       |              |       |          |
|-----------|-------|--------------|-------|----------|
| 2,808,388 | 10/57 | Hellman      | ----- | 260—29.6 |
| 3,069,390 | 12/62 | Kline et al. | ----- | 167—87.2 |
| 3,078,185 | 2/63  | Kine et al.  | ----- | 260—29.6 |

JULIAN S. LEVITT, *Primary Examiner.*